

Oct. 13, 1953

W. W. GULLETT

2,655,456

MANGANESE DIOXIDE FOR PRIMARY CELLS

Filed March 5, 1951



Fig. 1



INVENTOR

William W. Gullett

Fig. 2

## UNITED STATES PATENT OFFICE

2,655,456

## MANGANESE DIOXIDE FOR PRIMARY CELLS

William Waitman Gullett, College Park, Md., assignor to Manganese Battery Corporation, Riverdale, Md., a corporation

Application March 5, 1951, Serial No. 213,949

3 Claims. (Cl. 136—139)

1

This invention relates to the improvement of manganese dioxide for primary cells. It relates particularly to the improvement of bulk density of otherwise satisfactory battery oxide. It has for its aim the improvement of the bulk density of synthetic manganese dioxide without adversely affecting its depolarizing properties.

It is well known in the art that synthetic manganese dioxide such as that made by oxidizing manganese carbonate has good depolarizing properties but has a lower bulk density than natural African ore or battery oxide prepared by the electrolytic process. For example, the bulk density of synthetic chemical oxide varies from about 9–12 grams per cubic inch while natural electrolytic ore varies from 18–22 grams per cubic inch.

In this application the term "bulk density" will be used to designate the grams per cubic inch of the oxide as determined by the Scott volumeter.

The initial capacity of Le Clanche cells made from synthetic chemical oxide is less than that of cells made from electrolytic oxide substantially in proportion to the lower apparent density. I have found that if chemical synthetic oxides be densified in accordance with my invention that the initial capacity of Le Clanche cells made with them is increased in proportion to the density increase.

In Figure 1 there are illustrated typical discharge curves of Le Clanche cells. In this figure, curve A corresponds to a cell made with a synthetic oxide, and curve B, to an identical cell made with the same synthetic oxide densified in accordance with my invention. In Figure 2, comparative discharge curves are shown for identical alkaline cells. Curve B in this figure shows the discharge of a cell made with synthetic oxide, and curve A, the discharge of a cell made after densification of this oxide by the practice of my invention. Details of the construction of the cells of these illustrations will be found in Examples 1 and 3 respectively.

In carrying out the process of this invention I take synthetic chemical manganese dioxide and mix it with graphite. I then press the mixture at a temperature of 450–650° F., and a pressure of 10–50 tons per square inch. I then take the pellet so formed and crush it so that the product will pass a standard screen with 60 meshes to the linear inch and remain at least in substantial proportion on a standard screen with 200 meshes to the linear inch. The bulk density of such a product will be from 15–23 grams per cubic inch and will show on test in a Le Clanche cell an

2

improvement in initial capacity approximately proportional to the increase in bulk density.

I have found that the temperature and pressure of compacting the graphite-manganese dioxide mixture is critical. Even at the optimum temperature of 600° F. there is substantially no improvement with pressures below 10 tons per square inch. The maximum improvement in the range 450–650° F. is obtained at approximately 10 tons per square inch and at pressures above 50 tons per square inch there is a rapid falling off of the improvement in density.

There is substantially no improvement below 450° F. regardless of pressure and a rapid deterioration above 650° F. The maximum improvement is obtained at about 600° F. at all pressures within the range 10–50 tons per square inch.

The amount of graphite is also critical. The best results are obtained with 5% by weight of graphite. Smaller amounts down to 1% by weight give limited improvement and there is little or no improvement in density above 15% by weight of graphite.

The size of composite graphite-manganese dioxide particles produced by comminution is also critical. The maximum density is obtained with particles sized to pass a standard screen having 80 meshes to the linear inch and remain on one having 100 meshes. Particles intermediate in size between those which all remain on a screen having 60 meshes to the linear inch and those of such size that 80% by weight will remain on a screen having 200 meshes to the linear inch have a bulk density of more than the original unpressed manganese dioxide and are, therefore, within the scope of my invention.

The type of graphite used for the practice of my invention is important although good results can be obtained with any finely divided graphite. I prefer to use a micronized natural graphite.

Having now described the general principles of my invention, I will illustrate it by specific examples.

## Example I

45 I take synthetic manganese dioxide made by the oxidation of fully crystalline manganese carbonate and leaching with 10% sulphuric acid. This manganese dioxide has an analysis as follows:

|                                               |      |
|-----------------------------------------------|------|
| Available oxygen as per cent MnO <sub>2</sub> | 89.1 |
| Total manganese as per cent Mn                | 58.5 |
| Moisture as per cent H <sub>2</sub> O         | 1.9  |
| Iron as per cent Fe                           | 0.3  |
| Silica as per cent SiO <sub>2</sub>           | Nil  |
| pH                                            | 4.1  |

The crystal structure as determined by X-ray analysis was the so-called gamma. This material had a bulk density when measured on Scott volumeter of 12 grams per cubic inch. This material when made into Size AA Le Clanche cells showed a discharge through 300 ohms which has been plotted as curve *a*, Figure 1.

The same manganese dioxide was mixed with 5% by weight micronized graphite and hot-pressed at 600° F. and 40 tons per square inch. The pressure was applied only instantaneously. The pellet produced in this way was cooled and comminuted to the following sieve analysis:

70% of the material would pass a screen with 100 meshes to the linear inch but not one with 125 meshes.

20% of the material would pass a screen with 125 meshes to the linear inch but not one with 150 meshes.

7% of the material would pass a screen with 150 meshes to the linear inch but not one with 200 meshes.

3% passed through a screen with 200 meshes to the linear inch.

This material showed a bulk density of 22.1 grams per cubic inch when tested in the Scott volumeter.

This material was then made into identical Le Clanche cells and subjected to the same test as the unpressed manganese dioxide. The discharge curve is shown in curve *b* of Figure 1.

The improvement of density and performance of the oxide treated in accordance with my invention is clear.

#### Example 2

I take manganese dioxide such as is commercially available as a by-product of saccharin manufacture. This material is of high purity and is substantially amorphous. The apparent bulk density of this product is 7-8 grams per cubic inch. This material is mixed with 10% by weight of micronized natural graphite and pressed at 500° F. and 15 tons per square inch. The resulting pellets are comminuted so that the composite particles will all pass a standard screen with 100 meshes to the linear inch and remain on one with 150 meshes to the linear inch. This sized product has bulk density of 16 grams per cubic inch. The initial capacity of identical Le Clanche cells made from the original oxide and the pressed and comminuted oxide have been determined, and on discharge to 0.8 volt the capacity of the cells made from the pressed and comminuted oxide is 1.82 times that of cells made from the original oxide.

#### Example 3

I take oxide like that used in Example 1 and mix with 15% by weight of Acheson artificial graphite powder. I press this material at 600° F. and 40 tons per square inch. The resulting pellets are comminuted so that all of the composite particles will pass a screen with 60 meshes to the linear inch but not one with 100 meshes. The bulk density of this product was 15 grams per cubic inch. The product is made into a de-

polarizer for an alkaline cell by mixing with 2% by weight of powdered natural graphite and cold-pressing into a ½" diameter steel can at 40 tons per square inch. The electrolyte used was 30% KOH and the anode a compressed pellet of granular amalgamated zinc. This cell was discharged through a constant resistance of 300 ohms. A discharge curve for such a cell is shown in curve *a* of Figure 2. In curve *b*, Figure 2, is shown the discharge curve of an identical cell made with the oxide as mixed with 15% Acheson artificial graphite powder and cold-pressed into the ½" diameter steel can at 40 tons per square inch. This cell was also discharged through a constant resistance of 300 ohms.

What is claimed is:

1. The method of producing composite particles of chemical synthetic manganese dioxide and graphite having a bulk density of 15-23 grams per cubic inch which includes the steps of mixing chemical synthetic manganese dioxide with 1-15% by weight graphite powder, pressing the mixture at a temperature between 400° F. and 650° F. and a pressure of 10-50 tons per square inch, cooling the pellet so formed, and comminuting it so that the resulting particles will all pass a standard screen having 60 meshes to the linear inch and at least 80% by weight of the particles will remain on a screen having 200 meshes to the linear inch.

2. The method of improving the bulk density of synthetic manganese dioxide without impairing its depolarizing properties which includes the steps of mixing chemical synthetic manganese dioxide with 1-5% by weight graphite powder, pressing the mixture at a temperature between 400° F. and 650° F. at a pressure of 10-50 tons per square inch, cooling the pellet so formed and comminuting it so that the resulting particles will all pass a standard screen having 60 meshes to the linear inch and at least 80% by weight of the particles will be larger in average diameter than the original manganese dioxide.

3. The method of making a depolarizer for primary cells which includes the steps of mixing synthetic manganese dioxide having a gamma structure with 1-5% powdered graphite, heating to 400-600° F., pressing the mixture while at this temperature at 10-40 tons per square inch, then comminuting the resultant pellet to obtain particles which will all pass a standard screen having at least 60 meshes to the linear inch.

WILLIAM WAITMAN GULLETT.

#### References Cited in the file of this patent

#### UNITED STATES PATENTS

| Number    | Name            | Date          |
|-----------|-----------------|---------------|
| 642,414   | Bachmann et al. | Jan. 30, 1900 |
| 1,272,406 | Ellis           | July 16, 1918 |
| 1,293,272 | Wells           | Feb. 4, 1919  |
| 1,296,700 | Ruhoff          | Mar. 11, 1919 |
| 1,637,433 | Yngve           | Aug. 2, 1927  |
| 1,724,886 | Peiler          | Aug. 13, 1929 |
| 2,091,569 | Ridgway et al.  | Aug. 31, 1937 |
| 2,208,185 | Goudge          | May 27, 1939  |
| 2,307,301 | Hileman         | Jan. 5, 1943  |